

1

3,294,537

LITH-TYPE EMULSIONS WITH ORGANOSILICONE  
BLOCK COPOLYMERS

Kirby M. Milton, Rochester, N.Y., assignor to Eastman Kodak Company, Rochester, N.Y., a corporation of New Jersey  
No Drawing. Filed Sept. 17, 1965, Ser. No. 488,244  
23 Claims. (Cl. 96—67)

This invention relates to photography and particularly to improved photographic silver-halide emulsions of the "lith-type."

Photographic films used in the graphic arts for making halftone or line images should be capable of producing extremely high contrast and good image sharpness. These factors contribute in the case of half-tone images to high dot quality, that is, to the production of half-tone dots of high density and sharpness.

Photographic elements of the "lith-type" typically comprise fine-grain, high-contrast silver halide emulsions whose halides contain at least 50 mole percent chloride, and which are processed customarily in alkaline hydroquinone developing solutions having very low concentration of free sulfite ion in order to produce the high contrast and high dot quality required for good quality halftone reproduction. Such developing solutions are unstable, having very short tray or tank life during exposure to air, so the solutions must be prepared fresh before they are to be used for processing.

Common photographic "lith-type" materials are deficient with respect to exposure and development latitude when such materials are processed in preferred lithographic developing solutions which contain low concentrations of sulfite ions. This deficiency causes the contrast and halftone dot quality of the image reproduction to be overly sensitive to development time. It also is manifested in a nonlinearity in the relationship between effective film speed and development time, causing unequal increases in effective film speed with equal increases in development time.

Advantages are gained by increasing the contrast and quality of "lith-type" emulsions by the use of high molecular weight polyethylene glycols, coupled with development in low-sulfite, pure hydroquinone developers.

In films containing polyethylene glycols and their derivatives, however, optimum quality is obtained over only a rather restricted development time range and at the sacrifice of effective speed. When the quantity of polyethylene glycol is increased, optimum dot quality is obtained over a broader development time range, but only with a concomitant decrease in effective film speed, emulsion hardness and evenness of development. Evenness of development is the property of an exposed photographic material to maintain good effective contrast and good halftone dot quality over a relatively wide range of development time.

With or without the use of polyethylene glycols, it has in the past been necessary to use pure hydroquinone developers of low free-sulfite ion content in order to obtain the high contrast and halftone dot quality desired. Such developers are unstable because of aerial oxidation of the developing agent in alkaline solution. If the sulfite level is increased to prevent this oxidation, the desired contrast and dot quality of the processed photographic material are lost. Hence, it has been necessary either to prepare the developing solution fresh or to use two solutions which are mixed just before use, one of which contains hydroquinone in a mildly acidic solution buffered to a low free-sulfite level with a sulfite donor, and the other of which contains alkali. Even so, such solutions are stable after mixing for only a limited time

2

in a tray or a tank due to aerial oxidation of the developing agent.

It would be desirable to have an improved "lith-type" photographic material which is advantageously developable in a more stable developing solution, and which, when processed in such solutions, exhibits good contrast and halftone quality over an extended range of development time and permits obtaining equal increases in effective speed for a given increase in development time.

I have found that the addition of certain water-soluble organosilicone block copolymers to chlorobromoiodide emulsions increases speed of development, contrast and halftone quality and that these increases are found over a greater development range than that afforded by the use of polyethylene glycols. Regardless of the concentrations of the silicone compounds of my invention used and regardless of the developing times used within a wide range, the increase in speed is found to be constant for a given increase in development time. Furthermore, by the use of these materials, sufficient free sulfite ion can be added to the developer to give a stable single solution; yet the contrast and halftone dot quality are as high as normally seen in emulsions containing polyethylene glycol and developed in a low sulfite, hydroquinone developer.

It is, therefore, an object of my invention to provide a photographic film which produces high contrast and high halftone dot quality even when developed with a developer solution having sufficiently high free-sulfite content to insure good stability upon prolonged exposure to air in tray or tank.

Another object is to provide a photographic element which is capable of producing high contrast, high quality halftone images over a relatively broad range of film exposure and development times.

Another object is to provide a photographic element which develops evenly.

Still other objects will become apparent from the following specification and claims.

These and other objects are accomplished according to my invention by the use of photographic elements comprising a support, at least one hydrophilic colloidal fine-grain photographic silver halide emulsion layer whose halide is comprised of at least 50 mole percent of chloride, and either contiguous to the silver halide or integral therewith, certain water-soluble silicone-containing polyalkylene block polymers.

Water-soluble organosilicone polyalkyleneoxide polymers used to advantage according to my invention include those disclosed in U.S. Patent No. 2,917,480, issued December 15, 1959, assigned to Union Carbide Corporation.

Polymers used advantageously according to my invention are of the type which are prepared by reacting a dialkyl siloxane with a compound of the following structure:



wherein Y is an organic radical having a valence of x, and wherein n is an integer, x is an integer greater than 1, the values of n and x are such that the molecular weight of the compound, exclusive of E, Y and R is between 800 and 3,000, and E is a polyoxyethylene chain constituting about 10-70 percent by weight of the compound, R is a hydrogen atom or the residue of an organic compound containing an active hydrogen atom, such as, an alkyl, carbonyl, or aryl carbonyl group, e.g., alcohols, amines, acids, amides, phenols, etc. The conventional alkaline, pure hydroquinone, low free-sulfite developer may be used to develop my exposed element. It is also advantageous to use a developer having from 10 to about 30 grams of an alkali sulfite per liter of the developer solution. When

my elements are developed in the preferred developer solutions, not only is the image contrast high and the dot quality excellent but this excellent quality is produced over a wide range of exposures and development times.

My elements are particularly valuable when developed with a stable dihydroxybenzene developer with a high free sulfite ion concentration in an alkaline solution. My elements provide the following advantages:

(1) More even rate of speed change with changes in development times which allows varying the development time systematically to control speed without sacrificing quality;

(2) Better "dot quality" over a wider range of development times and temperatures;

(3) Elimination of or reduction in development defects, such as, "drag lines" when the materials are developed in automatic roller transport processing equipment;

(4) High contrast and much better dot quality when stable developer solutions containing a high free-sulfite concentration, e.g., 10 to 30 grams of an alkali metal sulfite per liter of solution are used;

(5) Increased speed without loss of dot quality when an onium salt is incorporated in my light-sensitive emulsion layer, and still further advantages will be apparent from the specification and claims. It is unexpected that the immediate organosilicone block polymers would produce the above cited advantages since other silicone-containing chemicals are known to have detrimental effects on photographic silver halide emulsions.

The organosilicone block polymers used according to my invention are water soluble and are advantageously added in a water solution to the aqueous hydrophilic colloid (either with or without the silver halide) before it is coated. The organosilicone block polymers are used to advantage over a wide range of concentrations. The operable range of concentrations is from .001 to 1.00 gram of block polymer per mole of silver, while the preferred range is from 0.010 to 0.200 gram per mole of silver. The optimum concentration of a given block polymer used in my elements depends upon the results desired, the particular silver halide emulsion, the developer solution, etc., and is readily determined by methods well known in the art. The determination of the optimum concentration is preferably made by employing the organosilicone block polymer in the silver halide emulsion layer or in an adjacent hydrophilic colloid layer according to the element that is desired.

Typical fine grain silver halide emulsions used to advantage can be prepared as described by MacWilliam U.S. 2,756,148 issued July 24, 1956. These emulsions may be used without being sensitized; however, it is advantageous to spectrally sensitize them according to methods well known in the art to make them orthochromatically-sensitized or panchromatically-sensitized.

The silver halide is dispersed in hydrophilic colloid materials used as binders, including gelatin, collodion, gum arabic, cellulose ester derivatives, such as alkyl esters of carboxylated cellulose, hydroxy ethyl cellulose, carboxy methyl hydroxy ethyl cellulose, synthetic resins, such as the amphoteric copolymers described by Clavier et al. in U.S. Patent 2,949,442, issued August 16, 1960, polyvinyl alcohol, and others well known in the art. Examples of these polymeric gelatin substitutes are copolymers of allylamine and methacrylic acid; copolymers of allylamine, acrylic acid and acrylamide; hydrolyzed copolymers of allylamine, methacrylic acid and vinyl acetate; the copolymers of allylamine, methacrylic acid and acrylonitrile; alkyl acrylate-acrylic acid copolymers, e.g., copolymers of butyl acrylate-acrylic acid; etc.

When my organosilicone block polymers are incorporated in a layer adjacent to the silver halide emulsion layer instead of in the light-sensitive layer, any of the hydrophilic colloids described hereinbefore may be used to advantage as a binder for coating my polymers.

It is advantageous to add certain onium salts, such as,

quaternary ammonium salts, sulfonium salts and phosphonium salts to my light-sensitive emulsions in order to increase the photographic speed without adversely affecting the improved dot quality, contrast and evenness of development. Examples of quaternary ammonium salts include nonyl pyridinium perchlorate, hexoxymethyl pyridinium perchlorate, ethylene bis-dioxymethyl pyridinium perchlorate and others described by Carroll U.S. 2,271,623, issued February 3, 1942, hexadecamethylene-1,16-bis(pyridinium perchlorate), 9,16 - diaza-7,18-dioxa-8,17-dioxotetracosane - 1,24 - bis(pyridinium perchlorate), and others of Beavers et al. U.S. 2,944,898, issued July 12, 1960. Other examples include the onium salts of polyoxyalkylenes of Carroll et al. U.S. 2,944,902, issued July 12, 1960, the polyonium salts of Carroll et al. U.S. 2,288,226, issued June 30, 1942, such as bis(lauryl methyl sulfonium p-toluene sulfonate) 1,2-ethane, N,N'-trimethylene dioxymethyl pyridinium perchlorate, etc., the sulfonium salts of Carroll et al. U.S. 2,275,727, issued March 10, 1942, such as n-decyl dimethyl sulfonium p-toluene sulfonate, n-nonyl dimethyl sulfonium p-toluene sulfonate, etc., and the phosphonium salts of Carroll et al. U.S. 2,271,622, issued February 3, 1942, such as tetramethylene bis-triethyl phosphonium bromide, lauryltriethylphosphonium bromide, etc.

My light-sensitive emulsions can be coated to advantage on any of the conventional photographic supports, including glass, cellulose acetate, polystyrene, polyalkyleneterephthalate, etc. The organosilicone block polymers can be coated advantageously in the silver halide emulsion layer or in a hydrophilic colloid layer that is either under or over the silver halide emulsion layer so that the block polymer is contiguous to the silver halide.

Included among the organosilicone block polymers used to illustrate my invention are those which may be prepared by reacting a polypropylene oxide-polyethylene oxide block polymer with dimethyl siloxane to give a copolymer having the following general structure:



wherein  $a$  and  $b$  are positive integers,  $M$  is a polyethyleneoxy chain constituting approximately 10-70% by weight of  $[(\text{M})_{\text{a}} - (\text{N})_{\text{b}}]_{\text{y}}$ ,  $N$  is a polypropyleneoxy chain having a molecular weight between approximately 800 and 3000, and wherein  $x$ ,  $y$  and  $n$  are positive integers as shown in Table A.

TABLE A

| Compound | Ratio $y:x$ | $n$    | Percent Silicon |
|----------|-------------|--------|-----------------|
| A        | 2:1         | 7      | 9.3             |
| B        | 2:1         | 6      | 7.0             |
| C        | 4:1         | 3      | 8.0             |
| D        | 2:1         | 7      | 12.0            |
| E        | 2:1         | 8      | 13.0            |
| F        | 1.5:1       | 1 to 8 | 6.3             |
| G        | 1:1.5       | 2      | 1.4             |
| H        | 1:1.5       | 1      | .62             |
| I        | 1:1         | 1      | .2              |

For a more complete understanding of the nature and objects of the invention, reference should be made to the following examples.

## Example 1

A gelatino silver chlorobromoiodide emulsion containing approximately 90 mole percent chloride, 9 mole percent bromide, and 1 mole percent iodide was divided into separate portions and the organosilicone polymers indicated in Table A were respectively added to the individual portions. The resulting compositions were coated on separate pieces of polyalkyleneterephthalate film support at a coverage of 455 mg. of silver and 450 mg. of gelatin per square foot. Samples of each coating

were exposed on an intensity scale sensitometer and processed in a developer of the composition:

|                               | G.   |
|-------------------------------|------|
| Hydroquinone                  | 15.0 |
| Sodium formaldehyde bisulfite | 50.0 |
| Sodium carbonate              | 35.0 |
| Sodium bicarbonate            | 22.5 |
| Sodium sulfite                | 2.5  |
| Potassium bromide             | 0.75 |
| Water to make 1.0 l.          |      |

for 4½ minutes at a temperature of 68° F., fixed in a conventional sodium thiosulfate fixing bath, washed and dried. The polymers, their concentration in each coating as well as speed, effective contrast and dot quality of the

opment rate. The following tables illustrate this advantage. These coatings were made and processed as described in Example I.

TABLE II (a)

| 5  | Coating No.                    | Compound | Gm./Ag mole | Change in Relative Speed over a 3 min. Development Time |
|----|--------------------------------|----------|-------------|---------------------------------------------------------|
| 10 |                                |          |             |                                                         |
| 1  | Oleyl ether of PEG (see Ex. I) |          | 0.12        | 713                                                     |
| 2  | Compound A of Table A          |          | 0.06        | 176                                                     |

TABLE II(b)

| Coating No. | Compound                       | Gm./Ag mole | Mol. Wt. of PPO Block | Percent PEG | Percent Si | Change in relative speed over a 3 min. Development Time |
|-------------|--------------------------------|-------------|-----------------------|-------------|------------|---------------------------------------------------------|
| 1           |                                |             |                       |             |            |                                                         |
| 2           | Oleyl ether of PEG (see Ex. I) | .125        |                       | 100         |            | 877                                                     |
| 3           | Organosilicone                 | .200        | 2,300                 | 10          | 4.5        | 134                                                     |
| 3           | do                             | .200        | 2,300                 | 10          | 9.6        | 129                                                     |

processed coatings and evenness of development that were obtained are summarized in Table I.

TABLE I

| Coating No. | Compound            | Gm./Ag mole | Rel. Speed | Effective Contrast * | Halftone Dot Quality† | Evenness of Development‡ |
|-------------|---------------------|-------------|------------|----------------------|-----------------------|--------------------------|
| 1           | None                |             | 102        | 6.4                  | 1                     | .08                      |
| 2           | PEG ①               | .125        | 100        | 7.6                  | 3                     | .205                     |
| 3           | Cpd. B of Table A   | .030        | 67         | 14.5                 | 7                     | .035                     |
| 4           | Cpd. C of Table A   | .040        | 74         | 11.3                 | 7                     | .010                     |
| 5           | Cpd. D of Table A   | .050        | 63         | 12.7                 | 7                     | .025                     |
| 6           | Cpd. E of Table A   | .050        | 53         | 12.0                 | 8                     | .055                     |
| 7           | Cpd. F of Table A   | .040        | 42         | 11.3                 | 8                     | .055                     |
| 8           | Cpd. G of Table A   | .060        | 76         | 10.0                 | 6                     | .02                      |
| 9           | Cpd. H of Table A   | .030        | 65         | 13.0                 | 7                     | .03                      |
| 10          | Cpd. I of Table A   | .030        | 48         | 13.0                 | 7                     | .09                      |
| 11          | Organosilicone I ②  | .120        | 37         | 16.0                 | 9                     | .07                      |
| 12          | Organosilicone II ③ | .100        | 53         | 13.1                 | 7,                    | .06                      |

① PEG: Oleyl ether of polyethyleneglycol having a molecular weight of 1,540.

② Organosilicone I: A water-soluble polysiloxane composed of dimethylsilicone sections and polyether sections containing 6.5% by weight of silicone.

③ Organosilicone II: A water-soluble polysiloxane composed of dimethyl siloxane sections and block polymers of ethylene oxide and propyleneoxide, containing 8.2% by weight of silicone.

\*"Effective Contrast" in the tables is determined by drawing a straight line between the net optical densities of 0.1 to 2.4 on the log exposure axis and taking the tangent of the angle formed between the straight line and the log exposure axis.

†"Halftone Dot Quality"—Dot quality is a measure of the quality of the reproduction of a halftone image. "Lith-type" photographic elements exposed to a halftone image, and developed, produce areas commonly referred to as shadow dots and areas known as highlight areas. Intermediate between these two extremes are areas of varying size. The dot quality used herein is a measure of the areas referred to as 50% dots (i.e., ½ clear and ½ developed density) and is expressed in a progressive scale where 9 is excellent and 1 is extremely poor. A dot quality below 6 is generally not acceptable.

‡"Evenness of Development"—Ideally, the rate of change in the log of the speed with change in development time should equal a constant; that is:

$$\log \text{speed at time } t+1 - \log \text{speed at time } t = K$$

When the rate of change in the speed is plotted against the development time, the slope of the resultant curve will approach 0 as K approaches a constant value. Evenness of development is the slope of the plot of K against time. In Table I, evenness of development is expressed in this way. The smaller the number, the more even the development, indicating more even spacing between the sensitometric curves obtained for equal differences in development time.

The data in Table I show that my "lith" elements containing organosilicone block copolymers produced good image contrast, good dot quality, and good evenness of development. The element outside my invention, i.e., those containing oleyl ether of polyethyleneglycol produced very poor dot quality, poor contrast and very poor evenness of development.

#### Example II

By varying the concentration of the water-soluble polyalkylene oxide-dialkyl siloxanes, it also is possible to make materials having relatively small changes in speed with development time. This characteristic is particularly advantageous in automatic processing equipment where the activity of the developer may vary with aging or other variables may be present which affect the devel-

60 The coatings in the following examples were prepared like those previously described and were processed in a high sulfite pure hydroquinone "lith" developer of the following type which is more stable to oxidation than the low sulfite developers normally used, but which usually gives poorer dot quality.

#### HIGH SULFITE DEVELOPER

|                                   |    |     |
|-----------------------------------|----|-----|
| Hydroquinone                      | g  | 15  |
| Boric acid                        | g  | 5.5 |
| KBr                               | g  | 2.7 |
| 70 K <sub>2</sub> CO <sub>3</sub> | g  | 90  |
| K <sub>2</sub> SO <sub>3</sub>    | g  | 20  |
| Diethylene glycol                 | cc | 30  |
| H <sub>2</sub> O to 1000 cc.      |    |     |

The results tabulated in Table III below show how the dot quality is maintained better over the entire tonal scale when a water-soluble polypropylene oxide-dialkyl siloxane is added to the emulsion compared to the results obtained with a simple polyethylene oxide polymer. This comparison also shows that the silicone polymer

however, that the addition of an "onium" salt to the emulsion will increase the speed without adversely affecting the improved dot quality and contrast obtained from the addition of the preferred copolymer. The coatings in this example were processed for 2 1/4 minutes in the developer of Example I.

TABLE V

| Coating No. | Onium Salt                                       | Gm./Ag mole | Relative Speed | Effective Contrast | Dot Quality |
|-------------|--------------------------------------------------|-------------|----------------|--------------------|-------------|
| 1           | None                                             |             | 100            | 8.9                | 8           |
| 2           | N,N' ethylenedioxymethyl<br>iridium perchlorate. | .066        | 302            | 13.0               | 8           |

gives results better than those obtained with alkyleneoxide block copolymers not containing silicone. The development time was 1 1/4 minutes.

TABLE III

| Coating No. | Polymer             | Gm./Ag mole | Dot Quality     |          |             |
|-------------|---------------------|-------------|-----------------|----------|-------------|
|             |                     |             | High-light Dots | 50% Dots | Shadow Dots |
| 1           | PEG ①               | .115        | 6               | 6        | 6           |
| 2           | Block polymer ②     | .020        | 7               | 7 1/2    | 7 1/2       |
| 3           | Organosilicone II ③ | .100        | 7               | 8        | 8 1/2       |

① Polyethyleneglycol of Example I.

② A copolymer composed of blocks of polyethylene oxide and poly propyleneoxide having a total molecular weight of 2,000 and wherein the ratio by weight of said blocks is 60 to 40, respectively.

③ Organosilicone II (see Example I).

#### Example IV

The coatings in this example were prepared like those previously described and were processed in the developing solution of Example I. The results tabulated in Table IV below illustrate how the image quality obtained with coatings containing a silicone-containing polyethyleneoxy copolymer remains good over a long development range and that it is better than that obtained with the related block copolymer from which it was synthesized.

TABLE IV

| Coating No. | Polymer                      | Gm./Ag mole | Dot Quality for Various Dev. Times in Min. |       |       |       |
|-------------|------------------------------|-------------|--------------------------------------------|-------|-------|-------|
|             |                              |             | 2 1/4                                      | 2 3/4 | 3 1/4 | 3 3/4 |
| 1           | Block Copolymer of Ex. III ④ | 0.020       | 8 1/2                                      | 8 1/2 | 8     | 6 1/2 |
| 2           | Compound I of Table A ⑤      | .025        | 9                                          | 9     | 8 1/2 | 8     |

④ Compound I of Table A was synthesized from the Block Copolymer of Example III and a siloxane.

#### Example V

The following example illustrates the improvement obtained from the addition of a quaternary ammonium salt to a high-contrast silver chlorobromide emulsion containing .10 gm. of a water-soluble polyalkylene-oxide-dialkyl siloxane (organosilicone II of Example I). While these polymers give an improvement in dot quality and contrast, they tend to reduce speed. It has been found,

15 It can be seen from the above results that the addition of the quaternary ammonium salt increased the speed of the emulsion by about 300 percent with no loss in dot quality or contrast. Other onium salts, such as the quaternary ammonium, sulfonium, and phosphonium 20 salts, described in U.S. Patents 2,271,622, 2,275,727, 2,288,226, 2,944,898, 2,271,623, and 2,944,902 can be used with similar results.

#### Example VI

An emulsion as described in Example I was divided 25 into two portions one of which was retained as a control, while to the other portion were added, per mole of silver halide, .200 gm. of the organosilicone I of Example I. Both portions were then coated and processed according to the procedures in Example I.

30 The results are shown in Table VI.

TABLE VI

| Dev. Time | Effective Contrast |          | Dot Quality |          | Fog  |
|-----------|--------------------|----------|-------------|----------|------|
|           | Control            | Sample 1 | Control     | Sample 1 |      |
| 1 1/4'    | 8.0                | 10.0     | 6           | 8        | 0.01 |
| 2 1/4'    | 8.0                | 12.5     | 3           | 8        | 0.01 |
| 2 3/4'    | 7.5                | 13.8     | 1           | 9        | 0.01 |
| 3 1/2'    | 6.4                | 15.0     | 1           | 9        | 0.01 |
| 3 3/4'    | 6.4                | 16.0     | 1           | 8        | 0.01 |

<sup>1</sup> Control plus organosilicone I of Example I.

<sup>1</sup> TS=too slow.

35 55 This example illustrates the improved contrast and dot quality attainable in the presence of an organosilicone block polymer over a wide range of development time.

#### Example VII

An emulsion as described in Example I was divided 60 into equal parts. One was retained as a control and to the others were added the compounds as listed in Table VII. Each sample was coated and tested as in Example I. The results obtained are shown in Table VII.

TABLE VII

| Development Time                           | Effective Contrast |       |       |       | Dot Quality |       |       |       | Fog  |
|--------------------------------------------|--------------------|-------|-------|-------|-------------|-------|-------|-------|------|
|                                            | 1.75'              | 2.75' | 3.75' | 4.75' | 1.75'       | 2.75' | 3.75' | 4.75' |      |
| Control                                    | 7.9                | 6.2   | 6.0   | 5.5   | 3           | 1     | 1     | 1     | 0.01 |
| Control plus oleyl ether of Ex. I          | 12.0               | 13.0  | 9.8   | 6.2   | 8           | 4     | 1     | 1     | 0.01 |
| Control plus Silicone I of Ex. I (50 mg.)  | 13.0               | >16   | 16    | 9.0   | 8           | 9     | 8     | 6     | 0.01 |
| Control plus Silicone I of Ex. I (75 mg.)  | 16                 | >16   | >16   | >16   | 8           | 9     | 9     | 7     | 0.01 |
| Control plus Silicone I of Ex. I (100 mg.) | 15.5               | >16   | >16   | >16   | 8           | 9     | 9     | 7     | 0.01 |
| Control plus Silicone I of Ex. I (125 mg.) | 13.5               | 16    | >16   | >16   | 1 TS        | 9     | 9     | 8     | 0.01 |
| Control plus Silicone I of Ex. I (150 mg.) | 13.0               | >16   | >16   | >16   | 1 TS        | 9     | 9     | 8     | 0.01 |

<sup>1</sup> Control plus organosilicone I of Example I.

<sup>1</sup> TS=too slow.

This example shows the excellent contrast and dot quality attainable with an organosilicone compound over a wide range of concentration and development time with development in a common lithographic pure-hydroquinone, low-sulfite content developing solution.

### Example VIII

This is a repeat of Example VII. The results are recorded in Table VIII.

TABLE VIII

| Development Time.....                            | Effective Contrast |       |       |       | Dot Quality |       |       |       | Fog  |
|--------------------------------------------------|--------------------|-------|-------|-------|-------------|-------|-------|-------|------|
|                                                  | 1.75'              | 2.75' | 3.75' | 4.75' | 1.75'       | 2.75' | 3.75' | 4.75' |      |
| Control.....                                     | 7.5                | 6.1   | 6.3   | 6.4   | 6           | 4     | 1     | 1     | 0.01 |
| Control plus oleyl ether of Ex. I (50 mg.).....  | 10.5               | 7.5   | 5.5   | 5.0   | 8           | 7     | 3     | 1     | 0.01 |
| Control plus oleyl ether of Ex. I (100 mg.)..... | 12.5               | >16   | 14.0  | 9.0   | 8           | 8     | 5     | 3     | 0.01 |
| Control plus oleyl ether of Ex. I (125 mg.)..... | 9.5                | >16   | >16   | 9.5   | 7           | 8     | 6     | 3     | 0.01 |
| Control plus oleyl ether of Ex. I (150 mg.)..... | 11.8               | 15.0  | 16.0  | 13.0  | 8           | 9     | 6     | 4     | 0.01 |
| Control plus oleyl ether of Ex. I (200 mg.)..... | 8.2                | >16   | >16   | 13.2  | 7           | 9     | 8     | 5     | 0.01 |
| Control plus Silicone I of Ex. I (50 mg.).....   | 7.5                | 6.8   | 5.8   | 5.1   | 7           | 3     | 2     | 1     | 0.01 |
| Control plus Silicone I of Ex. I (100 mg.).....  | >16                | 15.5  | >16   | >16   | 8           | 8     | 8     | 7     | 0.01 |
| Control plus Silicone I of Ex. I (125 mg.).....  | 16.0               | >16   | >16   | >16   | 7           | 8     | 8     | 7     | 0.01 |
| Control plus Silicone I of Ex. I (150 mg.).....  | >16                | >16   | 16.0  | >16   | 8           | 9     | 9     | 8     | 0.01 |
| Control plus Silicone I of Ex. I (200 mg.).....  | 13.5               | 16.0  | >16   | >16   | 1 TS        | 9     | 9     | 9     | 0.01 |

<sup>1</sup> TS=too slow.

It is shown that at comparable concentrations of a polyethyleneglycol and an organosilicone, the latter maintains a superior quality with respect to effective contrast and halftone dot quality.

### Example IX

A coating containing 75 mg. of the organosilicone II

bromide, and 1 mole percent iodide. The emulsions were 30 coated on a polyalkylene-terephthalate film support at a coverage of 455 mg. of silver and 450 mg. of gelatin per square foot. Samples of each coating were exposed on an intensity scale sensitometer and processed in the developing solution of Example I for 4 1/4 minutes, fixed, washed, and dried with the indicated results. See Table X.

TABLE X

| Sample  | Polymer                              | Mol. Wt. of PPO Block | Percent PEO <sup>1</sup> | Percent Si       | Mg./Mole AS | Rel. Speed | Eff. Contr. | Halftone Dot Quality | Evenness of Devel. |
|---------|--------------------------------------|-----------------------|--------------------------|------------------|-------------|------------|-------------|----------------------|--------------------|
| 1.....  | Polyethyleneglycol of Example I..... | .....                 | 100                      | .....            | 125         | 100        | 6.5         | 1                    | .20                |
| 2.....  | Silicone polymer I.....              | 1,650                 | 20                       | 6.8              | 50          | 55         | 12.1        | 9                    | .06                |
| 3.....  | Silicone polymer II.....             | 1,650                 | 10                       | 20.4             | 100         | 45         | 7.8         | 8                    | .05                |
| 4.....  | Silicone polymer III.....            | 1,650                 | 10                       | 4.8              | 50          | 60         | 11.0        | 7                    | .07                |
| 5.....  | Silicone polymer IV.....             | 1,650                 | 80                       | 2.2              | 100         | 118        | 4.8         | 2                    | .27                |
| 6.....  | Silicone polymer V.....              | 3,250                 | 40                       | 3.7              | 100         | 110        | 5.1         | 1                    | .18                |
| 7.....  | Silicone polymer VI.....             | 3,250                 | 40                       | 8.5              | 100         | 97         | 4.3         | 1                    | .19                |
| 8.....  | Silicone polymer VII.....            | 1,650                 | 50                       | 6.9              | 50          | 87         | 4.9         | 7                    | .03                |
| 9.....  | Silicone polymer VIII.....           | 1,650                 | 50                       | 6.9              | 50          | 76         | 10.0        | 8                    | .06                |
| 10..... | Copolymer A <sup>2</sup> .....       | .....                 | 100                      | ( <sup>3</sup> ) | 50          | 135        | 3.4         | 1                    | .22                |
| 11..... | Copolymer B <sup>2</sup> .....       | .....                 | 100                      | ( <sup>3</sup> ) | 50          | 123        | 2.7         | 1                    | .09                |

<sup>1</sup> PEO=oleyl ether of polyethylene oxide, Mol. Wt.=1,540.

<sup>2</sup> Copolymer A=copolymer of Carbowax 4000 and polydimethyl siloxane. Copolymer B=copolymer of Carbowax 1000 and polydimethyl siloxane.

<sup>3</sup> Undetermined.

Results: The compound outside my invention, i.e., those contained in samples 1, 6, 7, 10 and 11 do not yield acceptable dot quality.

of Example I and a control containing 115 mg. of the oleyl ether of polyethylene glycol per silver mole were each developed to optimum contrast in a developer containing a high level of sulfite ion of the following composition:

|                             |      |     |
|-----------------------------|------|-----|
| Hydroquinone .....          | g--  | 15  |
| Boric acid .....            | g--  | 5.5 |
| Potassium bromide .....     | g--  | 2.7 |
| Potassium carbonate .....   | g--  | 90  |
| Potassium sulfite .....     | g--  | 20  |
| Diethylene glycol .....     | cc-- | 30  |
| Distilled water to 1 liter. |      |     |

The following contrasts were obtained:

|                                                  | Gamma |
|--------------------------------------------------|-------|
| Control+oleyl ether of polyethylene glycol ..... | 3.7   |
| Control+silicone II of Ex. I .....               | 12.2  |

The following example illustrates this synergism.

### Example XI

The following coatings were prepared and processed as described in previous examples. The coatings were developed for 3 1/4 minutes in the developing solution of Example I.

It also has been found that the addition of saponin to 60 silver halide emulsions containing polyalkylene oxide-dialkyl siloxane polymers results in a large increase in speed without a loss of the beneficial effects produced by these polymers. This is unexpected in view of the fact that the addition of saponin to an emulsion containing a simple polyethylene glycol polymer produced only a minor speed effect and the addition of saponin to an emulsion in the absence of any polymeric material of this type produces no sensitometric effect.

The following example illustrates this synergism.

TABLE XI

| Coating Number | Polymer                   | Mg. Polymer/<br>Ag mole | Mg. Saponin/<br>Ag mole | Rel. Speed | Eff. Contr. | Fog | Evenness of Development | DQ <sup>1</sup> |
|----------------|---------------------------|-------------------------|-------------------------|------------|-------------|-----|-------------------------|-----------------|
| 1              | None                      | None                    | 100                     | 2.6        | .01         | .07 | .07                     | 1               |
| 2              | do                        | 5.1                     | 89                      | 2.8        | .01         | .07 | .07                     | 3               |
| 3              | do                        | 10.2                    | 100                     | 2.6        | .01         | .05 | .05                     | 1               |
| 4              | PEO <sup>2</sup>          | 130                     | None                    | 100        | 12.8        | .01 | .14                     | 8               |
| 5              | PEO <sup>2</sup>          | 130                     | 5.1                     | 115        | 11.0        | .01 | .14                     | 7               |
| 6              | PEO <sup>2</sup>          | 130                     | 10.2                    | 141        | 10.0        | .01 | .15                     | 7               |
| 7              | Organosilicone I of Ex. I | 85                      | None                    | 100        | 9.0         | .01 | .07                     | 9               |
| 8              | Organosilicone I of Ex. I | 85                      | 5.1                     | 159        | 12.2        | .01 | .02                     | 9               |
| 9              | Organosilicone I of Ex. I | 85                      | 10.2                    | 240        | 12.0        | .01 | .01                     | 8               |

<sup>1</sup> DQ=Dot Quality.<sup>2</sup> PEO=oleyl ether of polyethylene oxide, M.W.=1540.

It will be appreciated that although the block copolymers of this invention are usefully incorporated in the photographic emulsion or in an adjoining insensitive layer, the block copolymers can be imbibed from a processing bath, it being required only that the block copolymer be present during development.

The invention has been described in detail with particular reference to preferred embodiments thereof, but it will be understood that variations and modifications can be effected within the spirit and scope of the invention as described hereinabove and as defined in the appended claims.

I claim:

1. A photographic silver halide emulsion in which the halide comprises at least 50 mole percent chloride, said emulsion containing a block copolymer comprising blocks of polyoxyethylene and polyoxypropylene, about 10 to about 70%, by weight, of said copolymer being polyoxyethylene and the average molecular weight of polyoxypropylene in said copolymer being in the range of about 800 to about 3,000, said block copolymer containing up to about 15 percent, by weight, of silicon atoms in the main polymer chain.

2. A photographic silver halide emulsion in which the halide comprises at least 50 mole percent chloride, said emulsion containing about .001 to about 1 gram, per mole of silver halide, of a block copolymer comprising blocks of polyoxyethylene and polyoxypropylene, about 10 to about 70% by weight of said copolymer being polyoxyethylene and the average molecular weight of polyoxypropylene in said copolymer being in the range of about 800 to about 3,000, said block copolymer containing up to about 15% by weight of silicon atoms in the main polymer chain.

3. A photographic silver halide emulsion in which the halide comprises at least 50 mole percent chloride, said emulsion containing a polymer prepared by reacting a dialkyl siloxane with a block copolymer comprising blocks of polyoxyethylene and polyoxypropylene, about 10 to about 70% by weight of said copolymer being polyoxyethylene and the average molecular weight of the polyoxypropylene in said copolymer being in the range of about 800 to about 3,000, said block copolymer having the formula:



where Y is an organic radical having a valence of x; n is an integer; x is an integer greater than 1, the values of n and x being such that the molecular weight of said copolymer exclusive of Y, E and R is in the range of about 800 to about 3,000; E being a polyoxyethylene chain constituting from about 10 to about 70% by weight of said copolymer and R is a hydrogen atom, an alkyl group, an alkyl carbonyl group or an aryl carbonyl group.

4. A photographic silver halide emulsion in which the halide comprises at least 50 mole percent chloride, said emulsion containing about .001 to about 1 gram per mole of silver halide, of a polymer prepared by reacting a dialkyl siloxane with a block copolymer comprising blocks of polyoxyethylene and polyoxypropylene, about 10 to

about 70% by weight of said copolymer being polyoxyethylene and the average molecular weight of the polyoxypropylene in said copolymer being in the range of about 800 to about 3,000, said block copolymer having the formula:



where Y is an organic radical having a valence of x; n is an integer; x is an integer greater than 1, the values of n and x being such that the molecular weight of said copolymer exclusive of Y, E and R is in the range of about 800 to about 3,000; E being a polyoxyethylene chain constituting from about 10 to about 70% by weight of said copolymer and R is a hydrogen atom, an alkyl group, an alkyl carbonyl group or an aryl carbonyl group.

5. A photographic silver halide emulsion in which the halide comprises at least 50 mole percent chloride, said emulsion containing about .001 to about 1 gram per mole of silver halide, of a block copolymer having the formula:



wherein a and b are positive integers, M is a polyethyleneoxy chain constituting about 10 to about 70% by weight of



45 N is a polypropyleneoxy chain having a molecular weight between about 800 and 3,000, and wherein x, y and n are positive integers.

6. A photographic silver halide emulsion in which the halide comprises at least 50 mole percent chloride, and incorporated in the said silver halide emulsion about .001 to about 1 gram per mole of silver halide of a water-soluble block copolymer having the formula:



wherein a and b are positive integers, M is a polyethyleneoxy chain constituting about 10 to about 70% by weight of



60 N is a polypropylene chain having a molecular weight between about 800 and 3,000, and wherein x, y and n are positive integers, and n has a value of 1 to 8.

7. A photographic silver halide emulsion in which the halide comprises at least 50 mole percent chloride, said emulsion containing about .001 to about 1 gram per mole of silver halide, of a water-soluble block copolymer having the following formula:



75 wherein a and b are positive integers, M is a poly-

ethyleneoxy chain constituting about 10 to about 70% by weight of



N is a polypropyleneoxy chain having a molecular weight between about 800 and 3,000, and wherein x, y and n are positive integers, and the ratio of x:y is from 2:1 to 1:1.

8. A photographic element comprising a support having thereon a photographic silver halide emulsion layer in which the halide comprises at least 50 mole percent chloride, said emulsion containing a water-soluble block copolymer comprising blocks of polyoxyethylene and polyoxypropylene, about 10 to about 70% by weight of said copolymer being polyoxyethylene and the average molecular weight of the polyoxypropylene in said copolymer being in the range of about 800 to 3,000, said block copolymer containing up to about 15 percent by weight of silicon atoms in the main polymer chain.

9. A photographic element comprising a support having thereon a photographic silver halide emulsion layer in which the halide comprises at least 50 mole percent chloride, said emulsion containing a polymer prepared by reacting a dialkyl siloxane with a water-soluble block copolymer comprising blocks of polyoxyethylene and polyoxypropylene, about 10 to about 70% by weight of said copolymer being polyoxyethylene and the average molecular weight of the polyoxypropylene in said copolymer being in the range of about 800 to 3,000, said block copolymer having the formula:



where Y is an organic radical having a valence of x; n is an integer; x is an integer greater than 1, the values of n and x being such that the molecular weight of said copolymer exclusive of Y, E and R is in the range of about 800 to 3,000; E being a polyoxyethylene chain constituting from about 10 to about 70% by weight of said copolymer and R is a hydrogen atom, an alkyl group, an alkyl carbonyl group or an aryl carbonyl group.

10. A photographic element comprising a support having thereon a silver halide emulsion in which the halide comprises at least 50 mole percent chloride, said emulsion containing about .001 to about 1 gram per mole of silver halide, of a polymer prepared by reacting a dialkyl siloxane with a water-soluble block copolymer comprising blocks of polyoxyethylene and polyoxypropylene, about 10 to about 70% by weight of said copolymer being polyoxyethylene and the average molecular weight of the polyoxypropylene in said copolymer being in the range of about 800 to about 3,000, said water-soluble block copolymer having the formula:



where Y is an organic radical having a valence of x; n is an integer; x is an integer greater than 1, the values of n and x being such that the molecular weight of said copolymer exclusive of Y, E and R is in the range of about 800 to about 3,000; E being a polyoxyethylene chain constituting from about 10 to about 70% by weight of said copolymer and R is a hydrogen atom, an alkyl group, an alkyl carbonyl group or an aryl carbonyl group.

11. A photographic element comprising a support having thereon a photographic silver halide emulsion layer in which the halide is at least 50 mole percent chloride, said support having thereon at least one other layer, and incorporated in at least one layer of said element, a water-soluble block copolymer comprising blocks of polyoxyethylene and polyoxypropylene, about 10 to about 70% by weight of said copolymer being polyoxyethylene and the average molecular weight of polyoxypropylene in said copolymer being in the range of about 800 to about 3,000, said block copolymer containing up to about 15% by weight of silicon atoms in the main polymer chain.

12. A photographic element comprising a support having

thereon a photographic silver halide emulsion in which the halide comprises at least 50 mole percent chloride, said support having thereon at least one other layer, and incorporated in at least one layer of said element, about

- 5 .001 to about 1 gram, per mole of silver halide, of a water-soluble block copolymer comprising blocks of polyoxyethylene and polyoxypropylene, about 10 to about 70% by weight of said copolymer being polyoxyethylene and the average molecular weight of polyoxypropylene in said copolymer being in the range of about 800 to about 3,000, said block copolymer containing up to about 15% by weight of silicon atoms in the main polymer chain.

13. A photographic element comprising a support having thereon a photographic silver halide emulsion layer in which the halide comprises at least 50 mole percent chloride, said support having thereon at least one other layer, and incorporated in at least one layer of said element a polymer prepared by reacting a dialkyl siloxane with a water-soluble block copolymer comprising blocks of polyoxyethylene and polyoxypropylene, about 10 to about 70% by weight of said copolymer being polyoxyethylene and the average molecular weight of the polyoxypropylene in said copolymer being in the range of about 800 to about 3,000, said block copolymer having the formula:



- where Y is an organic radical having a valence of x; n is an integer; x is an integer greater than 1, the values of n and x being such that the molecular weight of said copolymer exclusive of Y, E and R is in the range of about 800 to about 3,000; E being a polyoxyethylene chain constituting from about 10 to about 70% by weight of said copolymer and R is a hydrogen atom, an alkyl group, an alkyl carbonyl group or an aryl carbonyl group.

14. A photographic element comprising a support having thereon a photographic silver halide emulsion layer in which the halide comprises at least 50 mole percent chloride, said support having thereon at least one other layer, and incorporated in at least one layer of said element, about .001 to about 1 gram, per mole of silver halide, of a polymer prepared by reacting a dialkyl siloxane with a water-soluble block copolymer comprising blocks of polyoxyethylene and polyoxypropylene, about 10 to about 70% by weight of said copolymer being polyoxyethylene and the average molecular weight of the polyoxypropylene in said copolymer being in the range of about 800 to about 3,000, said block copolymer having the formula:



- where Y is an organic radical having a valence of x; n is an integer; x is an integer greater than 1, the values of n and x being such that the molecular weight of said copolymer exclusive of Y, E and R is in the range of about 800 to about 3,000; E being a polyoxyethylene chain constituting from about 10 to about 70% by weight of said copolymer and R is a hydrogen atom, an alkyl group, an alkyl carbonyl group or an aryl carbonyl group.

15. A photographic silver halide emulsion in which the halide comprises at least 50 mole percent chloride, said emulsion containing about .001 to about 1 gram, per mole of silver halide, of a water-soluble block copolymer comprising blocks of polyoxyethylene and polyoxypropylene, about 10 to about 70% by weight of said copolymer being polyoxyethylene and the average molecular weight of polyoxypropylene in said copolymer being in the range of about 800 to about 3,000, said block copolymer containing up to about 15% by weight of silicon atoms in the main polymer chain, said emulsion containing a compatible speed increasing onium salt.

16. A photographic silver halide emulsion in which the halide comprises at least 50 mole percent chloride, said emulsion containing a polymer prepared by reacting a dialkyl siloxane with a water-soluble block copolymer comprising blocks of polyoxyethylene and polyoxypropyl-

ene, about 10 to about 70% by weight of said copolymer being polyoxyethylene and the average molecular weight of the polyoxypropylene in said copolymer being in the range of about 800 to about 3,000, said water-soluble block copolymer having the formula:



where  $Y$  is an organic radical having a valence of  $x$ ;  $n$  is an integer;  $x$  is an integer greater than 1, the values of  $n$  and  $x$  being such that the molecular weight of said copolymer exclusive of  $Y$ ,  $E$  and  $R$  is in the range of about 800 to about 3,000;  $E$  being a polyoxyethylene chain constituting from about 10 to about 70% by weight of said copolymer and  $R$  is a hydrogen atom, an alkyl group, an alkyl carbonyl group or an aryl carbonyl group, said emulsion containing a compatible speed-increasing onium salt.

17. A photographic element comprising a support having thereon a silver halide emulsion in which the halide comprises at least 50 mole percent chloride, said emulsion containing about .001 to about 1 gram per mole of silver halide, of a water-soluble block copolymer having the formula:



wherein  $a$  and  $b$  are positive integers,  $M$  is a polyethylenoxy chain constituting about 10 to about 70% by weight of



$N$  is a polypropyleneoxy chain having a molecular weight between about 800 and 3,000, and wherein  $x$ ,  $y$  and  $n$  are positive integers.

18. A photographic element comprising a support having thereon a photographic silver halide emulsion in which the halide comprises at least 50 mole percent chloride, said support having thereon at least one other layer, and incorporated in at least one layer of said element, about .001 to about 1 gram per mole of silver halide of a water-soluble block copolymer having the formula:



wherein  $a$  and  $b$  are positive integers,  $M$  is a polyethylenoxy chain constituting about 10-70% by weight of



$N$  is a polypropyleneoxy chain having a molecular weight between about 800 and 3,000, and wherein  $x$ ,  $y$  and  $n$  are positive integers.

19. A photographic element comprising a support having thereon a silver halide emulsion in which the halide comprises at least 50 mole percent chloride, said emulsion

containing about .001 to about 1 gram per mole of silver halide, of a water-soluble block copolymer having the following formula:



wherein  $a$  and  $b$  are positive integers,  $M$  is a polyethylenoxy chain constituting about 10-70% by weight of



$N$  is a polypropyleneoxy chain having a molecular weight between about 800 and 3,000, and wherein  $x$ ,  $y$  and  $n$  are positive integers and the ratio of  $x:y$  is from 2:1 to 1:1.

15 20. An element of claim 19 in which  $n$  has a value of one to eight.

21. A process of developing an exposed photographic silver halide emulsion in which the halide comprises at least 50 mole percent chloride, comprising imbibing into the said emulsion a block copolymer comprising blocks of polyoxyethylene and polyoxypropylene, about 10 to about 70%, by weight, of said copolymer being polyoxyethylene and the average molecular weight of polyoxypropylene in 20 said copolymer being in the range of about 800 to about 3,000, said block copolymer containing up to about 15 percent, by weight of silicon atoms in the main polymer chain, and reducing the exposed silver halide to silver by means of a silver halide reducing agent.

22. A photographic silver halide emulsion in which the halide comprises at least 50 mole percent chloride, said emulsion containing saponin and a block copolymer comprising blocks of polyoxyethylene and polyoxypropylene, about 10 to about 70% by weight of said copolymer being polyoxyethylene and the average molecular weight of polyoxypropylene in said copolymer being in the range of about 800 to about 3,000, said block copolymer containing up to about 15% by weight of silicon atoms in the main polymer chain.

23. A photographic silver halide emulsion in which the halide comprises at least 50 mole percent chloride, said emulsion containing saponin and a block copolymer comprising blocks of polyoxyethylene and polyoxypropylene, about 10 to about 70% by weight of said copolymer being polyoxyethylene and the average molecular weight of polyoxypropylene in said copolymer being in the range of about 800 to about 3,000, said block copolymer containing up to about 15% by weight of silicon atoms in the main polymer chain, said emulsion containing a compatible speed-increasing onium salt.

No references cited.

NORMAN G. TORCHIN, Primary Examiner.

55 J. RAUBITSCHEK, Assistant Examiner.